

# UNITED STATES PATENT OFFICE.

AMBROSE J. MANDELL, OF MORRISTOWN, NEW JERSEY, ASSIGNOR TO ELECTRICAL ALLOY COMPANY, OF MORRISTOWN, NEW JERSEY, A CORPORATION OF NEW JERSEY.

## METALLIC ALLOY.

1,403,558.

Specification of Letters Patent. Patented Jan. 17, 1922.

No Drawing.

Application filed January 29, 1920. Serial No. 354,889.

To all whom it may concern:

Be it known that I, AMBROSE J. MANDELL, a citizen of the United States, residing at Morristown, in the county of Morris and 5 State of New Jersey, have invented certain new and useful Improvements in Metallic Alloys, of which the following is a specification.

This invention relates to an improved 10 metal alloy, and has for its primary object to provide a composition consisting of several metallic ingredients proportioned in such a manner as to produce a metal alloy which is characterized by high electrical 15 resistance properties; great resistance to corrosion and oxidation and possessing high tensile strength.

With the above and other objects in view as will become apparent as the description 20 proceeds, the invention consists in the combination of the several metallic ingredients hereinafter specified.

The constituents of my improved alloy are as follows and may vary by weight between 25 the limits stated:

|                 |        |
|-----------------|--------|
| Nickel -----    | 40-65% |
| Copper-----     | 20-30% |
| Iron -----      | 02-15% |
| Manganese ----- | 02-25% |

Metal alloy having the metallic ingredients in the relative proportions specified has 30 higher electrical resistant properties than what is known as "Monel" metal, upon 35 which my invention is an improvement. I have found that the electrical resistance of Monel metal is very little affected by relatively great changes in the proportions of nickel and copper present in the alloy, but is 40 very greatly affected by small variations in the percentages of iron, manganese and similar metals, which are usually present in quantities not exceeding 2%.

Therefore, by increasing the iron or manganese content or both in suitable proportions, I have found that the electrical resistance of the resultant alloy may be greatly increased. Either iron or manganese may be added alone, or commercial ferromanganese of suitable percentages may be added, 50 depending on the properties desired in the resulting alloy.

The addition of iron greatly increases the electrical resistance of the resultant alloy,

but somewhat lowers its resistance to corrosion, and I have found that if there is an excess iron content, the hardness of the alloy is unduly increased, thus making it difficult to work. The manganese increases both the electrical resistance and hardness of the 55 alloy but does not greatly change the resistance to corrosion. Therefore, very much more manganese than iron may be added without making the alloy too difficult to work.

Monel metal possesses the following constituents in approximately the proportions set forth:

|                         |     |
|-------------------------|-----|
| Nickel -----            | 67% |
| Copper-----             | 28% |
| Iron and manganese----- | 5%  |

I have found wide variations in the electrical resistance of Monel metal due to non-uniform composition and that such variations can be almost eliminated in the alloy produced after the addition of iron, manganese or ferromanganese in quantities calculated from the composition of the Monel metal used, so as to have the percentages of 75 iron and manganese in the resulting alloy, constant within limits.

The percentage of iron which may be allowed in the resulting material after proper additions, without making the alloy 80 too hard and brittle for working by customary methods is 15%, while the percentage of manganese which may be allowed is 25%.

After adding iron, manganese or ferromanganese to the Monel metal, for the purpose of increasing the electrical resistance, a series of alloys can be produced having specific electrical resistance in excess of 300 ohms per circular mil-foot, and in some cases in excess of 500 ohms per circular mil-foot, and the alloys are very strong, can be worked by ordinary and well-known metal-working methods, can be easily cast, and have properties very similar to those of Monel metal with regard to resistance to 90 corrosion, erosion and oxidation, besides having a much greater electrical resistance than that of Monel metal.

Such series of alloys I have found possess high electrical resistance varying from approximately 30 to 50 times that of copper, depending on the composition; high tensile strength, when drawn, being in excess of 105

100,000 pounds per square inch; resistance to corrosion, especially that due to atmospheric influences. Nickel-steel and similar steel alloys, having approximately 5 the same electrical resistance, all corrode seriously in air, and in this respect, the alloys described are a very great improvement thereover.

The alloys described all strongly resist 10 oxidation at temperatures below a bright red heat, about 600° centigrade.

The new composition constituting my invention may be put to many practical purposes advantageously and it is especially 15 adaptable for electrical heating or resistance purposes, although manifestly it may be put to mechanical purposes where circumstances might make it desirable, since the resulting alloy may be cast, drawn, rolled, forged or 20 machined, and possesses in addition great strength, non-corroding and durability.

Having thus described my invention what I claim as new herein and desire to secure by Letters Patent is:

25 1. An alloy for electrical-resistance elements consisting of nickel, copper, iron, and manganese, the iron content being greater than 2% and the manganese content being within the limits of 2% and 25% by weight.

30 2. An alloy for electrical-resistance elements consisting of nickel, copper, manganese, and iron, the manganese content being greater than 2% and the iron content being within the limits of 2% and 15% by weight.

35 3. An alloy for electrical-resistance elements consisting of copper, iron, manganese and nickel, the iron and manganese content being each greater than 2% and the nickel content being within the limits of 40% and 40 65% by weight.

4. An alloy for electrical-resistance elements consisting of nickel, iron, manganese, and copper, the combined iron and manganese content being not less than 5% and the copper being within the limits of 20% and 45 30% by weight.

5. An alloy for electrical-resistance elements consisting of nickel, copper, from 2% to 15% by weight of iron and 2% to 25% 50 by weight of manganese.

6. An alloy for electrical-resistance elements consisting of nickel, from 20% to 30% by weight of copper, 2% to 15% by weight of iron and 2% to 25% by weight 55 of manganese.

7. An alloy for electrical-resistance elements consisting of copper, from 40% to 65% by weight of nickel, 2% to 15% by weight of iron and 2% to 25% by weight of 60 manganese.

8. An alloy for electrical-resistance elements consisting of from 40% to 65% by weight of nickel, 20% to 30% by weight of copper, 2% to 15% by weight of iron and 65 2% to 25% by weight of manganese.

9. A composition of matter consisting of copper, iron, manganese and not more than 65% by weight of nickel, the combined percentage of iron and manganese being not less than 5%. 70

10. A composition of matter consisting of nickel, copper, iron and manganese, the latter exceeding 2% by weight and the combined percentage of manganese and iron being not less than 5%. 75

11. A composition of matter consisting of nickel, copper, manganese and iron, the latter exceeding 2% by weight and the combined iron and manganese content being not less than 5%. 80

12. A composition of matter consisting of nickel, copper, iron and manganese, the iron being equal to about 2% or more and the manganese exceeding 2% by weight but not exceeding 25% by weight. 85

13. A composition of matter consisting of nickel, copper, manganese and iron, the manganese being equal to about 2% or more and the iron exceeding 2% but not exceeding 15% by weight. 90

14. An alloy consisting of nickel, copper, iron and manganese, the percentage by weight of the latter two combined being from 5% to 40%, but neither less than 2%, said alloy having high electrical resistance, 95 high tensile strength and being strongly resistant to corrosion and oxidation, substantially as described.

15. An electrical-resistance alloy consisting of nickel not less than 40% by weight, copper not less than 20% by weight, iron over 2% up to 15% by weight, and manganese not less than 2% by weight. 100

16. An electrical-resistance alloy consisting of nickel not greater than 65% by weight, copper not greater than 30% by weight, iron not greater than 15% by weight, and manganese not greater than 25% by weight, neither the iron nor the manganese being less than 2% and the combined percentage thereof being not less than 5%. 110

17. An electrical-resistance alloy consisting of nickel, copper, iron and manganese the nickel and copper combined being not less than 60% by weight and not more than 95% by weight, the iron and manganese combined being greater than 4% by weight and not more than 40% by weight. 115

18. An alloy similar to Monel metal but having any desired electrical resistivity higher than that of Monel metal up to about 500 ohms per circular mil-foot, said alloy being composed of nickel, copper, manganese and iron, the combined percentage of manganese and iron being greater than that of Monel metal and equal to a value dependent upon the resistivity desired to be obtained, at least one of said last-mentioned ingredients being present to a value not less than 3½%. 120

19. An alloy having high resistivity to the electrical current and composed of nickel, copper, manganese and iron, the percentage of manganese and iron combined exceeding 5 that of Monel metal by a quantity dependent upon the electrical resistivity which it is desired to impart to the alloy.
20. An alloy composed of the same ingredients as Monel metal and having substantially the same properties, but containing 10 iron and manganese together in proportion above that of Monel metal to render the alloy of high resistance to electrical current.

AMBROSE J. MANDELL.